

Dec. 19, 1933.

E. H. NOLLAU ET AL

1,940,462

COATED FABRICS

Filed Sept. 27, 1930



- 1 Dyed Fabric
- 2 Cellulose nitrate, softner, pigment, coating composition
- 3 Adhesive
- 4 Fabric backing
- 5 Cellulose nitrate, wax, softner, coating composition

*Edgar H. Nollau  
Donald A. Rankin* INVENTORS

BY THEIR ATTORNEY  
*Ralph F. Miller*

## UNITED STATES PATENT OFFICE

1,940,462

## COATED FABRIC

Edgar H. Nollau and Donald A. Rankin, Newburgh, N. Y., assignors to E. I. du Pont de Nemours & Company, Wilmington, Del., a corporation of Delaware

Application September 27, 1930  
Serial No. 484,860

12 Claims. (Cl. 154—46)

This invention relates to coated fabrics and more particularly to such products adapted to serve as leather substitutes. This invention has as an object the production of a coated fabric product. A further object is the production of a leather substitute which is of decorative appearance and of general utility in the arts. A still further object is to impart certain desirable properties to fabrics which they do not naturally possess. Other objects will appear hereinafter.

The objects are accomplished by the following preferred mode of procedure which will be described in connection with the figure in the drawing showing a section of the preferred form of our coated fabric product.

A woven sheeting 1, preferably one of such a weight to be equivalent to approximately 2.5 yards per pound per 58" in width, is dyed, by the usual method of jig or pad dyeing, a color approximating the color of the finished product, this color being determined by the pigment in the coating composition next applied. This fabric may be a plain weave fabric, such as for instance, a sheeting, or other types of weaves, as drills, etc. After the material is dyed and carefully dried, it is coated in a suitable machine by means of a doctor knife having a sharp edge with two coats of a pigmented cellulose nitrate-softener composition of the approximate following formula:

|                   | Per cent |
|-------------------|----------|
| Cellulose nitrate | 26-23    |
| Softener          | 46-52    |
| Pigment           | 28-25    |

The softener may be either raw castor oil, blown castor oil, or other common softeners, used in cellulose nitrate coating compositions. Following these two coats, two additional coats of the same material are applied with a doctor knife having a dull edge. This coating comprised of cellulose nitrate, softener and pigment is designated by the numeral 2 in the drawing. The material is then embossed by the usual press or roller embossing equipment in the grain which is desired in the ultimate finished product. If it is desired to produce a two-tone effect in the finished product, the material after embossing is treated with a composition similar to that noted above but usually in a contrasting color in order to give the final two-tone effect. This coated material is then combined by the usual doubling or combining operation to another fabric 4, either a sheeting, drill, sateen, or heavier

fabric, by means of a suitable adhesive, as for instance, rubber cement 3. The adhesive is applied to both fabrics and then the fabrics combined by passing thru the doubling machine. The rubber cement may be replaced by other suitable adhesives, such as pyroxylin compositions, and treated oil compositions, etc.

A special coating 5 comprised of the following ingredients is now applied to the surface of coating 2.

|                         | Per cent |
|-------------------------|----------|
| Cellulose nitrate       | 10.8     |
| Ceresin wax (refined)   | 2.7      |
| Dibutyl phthalate       | 10.8     |
| Ethyl acetate C. P.     | 17.3     |
| Denatured ethyl alcohol | 33.6     |
| Toluol C. P.            | 24.8     |

Dry solids in these compositions vary between 12 and 28%. If desired, however, the compositions may be further diluted with such materials as toluol, benzol, or gasoline. These ingredients are preferably compounded in the following manner: The ceresin wax, after being liquefied by heating, is carefully mixed with warm toluol by thorough agitation. To this solution of the wax is added a cellulose nitrate dispersion in a solvent consisting of ethyl acetate and denatured alcohol in a concentration of approximately 17%. The mixture is carefully stirred until an even and perfectly smooth dispersion is obtained. The dibutyl phthalate is then added with constant stirring. After the coating 5 of this composition is applied, a special lustrous finish may be obtained by further embossing.

The ratio of the ingredients in the above mentioned coating composition from which the coating 5 is obtained, may vary somewhat from the values indicated. Thus, the cellulose nitrate may vary between 5 and 15%, the ceresin wax from 1 to 9.5%, the dibutyl phthalate from 5 to 15%, the ethyl acetate from 16 to 21%, the denatured ethyl alcohol from 28 to 36%, and the toluol from 20 to 35%. These ingredients may also be substituted by equivalents as will be understood by those skilled in the art. Suitable wax-like substances that may replace the ceresin wax mentioned in the example are as follows: carnauba wax, candelilla wax, paraffin wax, or similar straight chain hydrocarbon waxes, solid hydrocarbon waxes of the cyclic type, Japan wax, Montan wax, spermaceti wax, hydrogenated castor oil, and resins of the polyhydric alcohol-polybasic acid type.

These resins, as understood by those skilled

in the art, are the reaction products of polyhydric alcohols (as glycerol) with polybasic acids (as phthalic anhydride) in which drying oils, oil acids, or other modifying and solubilizing agents have been incorporated. Suitable softening agents, other than dibutyl phthalate, may be exemplified by: dibutyl tartrate, tricresyl phosphate, raw castor oil, blown castor oil, and blown cotton seed oil. Various organic solvents may 10 replace those mentioned, as for instance, acetone, butyl acetate, ethyl propionate, methyl alcohol, benzol, and xylene.

While it is desirable to interpose the coating 2 composed of cellulose nitrate, softener and 15 pigment between the final or outside coating comprised of the ingredients referred to above, it is to be understood that a valuable coated fabric product is obtained by applying the coating 5 directly to the base material 1. The treatment 20 herein disclosed results in the production of a film on either coated or uncoated fabric which is discontinuous with respect to the principal ingredient, namely, cellulose nitrate. The exceptional 25 properties which characterize our improved product are due to the existence of this discontinuous type of film. Among the properties referred to may be mentioned the extremely high exudation temperatures and low cold crack temperatures. It is preferred, however, to make the 30 product as indicated in the drawing because of the leather-like and attractive finish imparted to the composite product by the coating 2.

A coated fabric product made in accordance with the present invention possesses several valuable 35 characteristics. The product has soil resistance; that is, dust and dirt do not adhere to the surface as in the case of regular fabrics. Oil and grease do not penetrate the surface as is the case with untreated fabrics. The product is also 40 washable in that dust and dirt, as well as oil and grease can be satisfactorily removed by the usual cleaning agents without harming the fabric. Since the product is water repellent, the material does not absorb water as untreated fabrics 45 do, and the material, therefore, shows little tendency to shrink. The treatment also appreciably reduces the tendency of the fabric to fade.

As many apparently widely different embodiments of this invention may be made without 50 departing from the spirit and scope thereof, it is to be understood that we do not limit ourselves to the specific embodiments thereof except as defined in the appended claims.

We claim:

1. A washable, oil and grease resistant, coated 55 fabric comprising a textile fabric carrying a film comprising cellulose nitrate, a wax, and a softener which is a non-solvent for the wax, the character and proportion of the ingredients being such that the film is discontinuous with respect to the cellulose nitrate.

2. A washable, oil and grease resistant, coated 60 fabric comprising a textile fabric carrying a film comprising, by weight, 5-15 parts of cellulose nitrate, 1-9.5 parts of a wax, and 5-15 parts of a softener which is a non-solvent for the wax, the character of the ingredients being such that the film is discontinuous with respect to the cellulose nitrate.

3. A washable, oil and grease resistant, coated 70 fabric comprising a textile fabric carrying a film comprising, by weight, 5-15 parts of cellulose nitrate, 1-9.5 parts of ceresin wax, and 5-15 parts of a softener which is a non-solvent for the ceresin wax, the character of the ingredients

being such that the film is discontinuous with respect to the cellulose nitrate.

4. A washable, oil and grease resistant, coated 80 fabric comprising a textile fabric carrying a film comprising, by weight, 10.8 parts cellulose nitrate, 10.8 parts dibutyl phthalate, and 2.7 parts ceresin wax, the character of the ingredients being such that the film is discontinuous with respect to the cellulose nitrate.

5. A washable, oil and grease resistant, coated 85 fabric comprising a textile fabric, a film comprising cellulose nitrate, a softener and a pigment superposed on said fabric and a surface film comprising cellulose nitrate, a wax, and a softener which is a non-solvent for the wax, superposed on said first film, the character and proportion of the ingredients in said surface film being such that the film is discontinuous with respect to the cellulose nitrate.

6. A washable, oil and grease resistant, coated 90 fabric comprising a textile fabric, a film comprising cellulose nitrate, a softener and a pigment superposed on said fabric and a surface film comprising, by weight, 5-15 parts of cellulose nitrate, 1-9.5 parts of a wax, and 5-15 parts of a softener which is a non-solvent for the wax, superposed on said first film, the character of the ingredients in said surface film being such that the film is discontinuous with respect to the cellulose nitrate.

7. A washable, oil and grease resistant, coated 95 fabric comprising a textile fabric, a film comprising cellulose nitrate, a softener and a pigment superposed on said fabric and a surface film comprising, by weight, 5-15 parts of cellulose nitrate, 1-9.5 parts of ceresin wax, and 5-15 parts of a softener which is a non-solvent for the ceresin wax, superposed on said first film, the character of the ingredients in said surface film being such that the film is discontinuous with respect to the cellulose nitrate.

8. A washable, oil and grease resistant, coated 100 fabric comprising a textile fabric, a film comprising cellulose nitrate, a softener and a pigment superposed on said fabric and a surface film comprising, by weight, 10.8 parts cellulose nitrate, 10.8 parts dibutyl phthalate, and 2.7 parts ceresin wax superposed on said first film, the character 105 of the ingredients in said surface film being such that the film is discontinuous with respect to the cellulose nitrate.

9. A washable, oil and grease resistant, artificial 110 leather comprising a relatively heavy fabric base, a lighter fabric cemented to one face of said fabric base, a film comprising cellulose nitrate, a softener, and a pigment superposed on said lighter fabric, and a surface film comprising cellulose nitrate, a wax, and a softener which is a non-solvent for the wax, superposed on said first film, the character and proportion of the ingredients 115 in said surface film being such that the film is discontinuous with respect to the cellulose nitrate.

10. A washable, oil and grease resistant, artificial 120 leather comprising a relatively heavy fabric base, a lighter fabric cemented to one face of said fabric base, a film comprising cellulose nitrate, a softener, and a pigment superposed on said lighter fabric, and a surface film comprising, by weight, 5-15 parts of cellulose nitrate, 1-9.5 parts of a wax, and 5-15 parts of a softener which is a non-solvent for the wax, superposed on said first film, the character of the ingredients in said surface film being such that the film is discontinuous with respect to the cellulose nitrate.

11. A washable, oil and grease resistant, arti- 125

130

135

140

145

150

ficial leather comprising a relatively heavy fabric base, a lighter fabric cemented to one face of said fabric base, a film comprising cellulose nitrate, a softener, and a pigment superposed on said lighter fabric, and a surface film comprising, by weight, 5-15 parts of cellulose nitrate, 1-9.5 parts of ceresin wax, and 5-15 parts of a softener which is a non-solvent for the ceresin wax, superposed on said first film, the character of the ingredients in said surface film being such that the film is discontinuous with respect to the cellulose nitrate. 80

10 in said surface film being such that the film is discontinuous with respect to the cellulose nitrate. 85

12. A washable, oil and grease resistant, artificial leather comprising a relatively heavy fabric

EDGAR H. NOLLAU.  
DONALD A. RANKIN.

15 90

20 95

25 100

30 105

35 110

40 115

45 120

50 125

55 130

60 135

65 140

70 145

75 150